



US009017239B2

(12) **United States Patent**  
**Ishida et al.**

(10) **Patent No.:** **US 9,017,239 B2**  
(45) **Date of Patent:** **Apr. 28, 2015**

(54) **ELECTROPHOTOGRAPHIC MEMBER,  
PROCESS CARTRIDGE AND  
ELECTROPHOTOGRAPHIC APPARATUS**

(75) Inventors: **Kazutoshi Ishida**, Mishima (JP);  
**Hiidenori Satoh**, Odawara (JP); **Tomoya Uesugi**, Susono (JP)

(73) Assignee: **Canon Kabushiki Kaisha**, Tokyo (JP)

(\*) Notice: Subject to any disclaimer, the term of this patent is extended or adjusted under 35 U.S.C. 154(b) by 294 days.

(21) Appl. No.: **13/615,433**

(22) Filed: **Sep. 13, 2012**

(65) **Prior Publication Data**

US 2013/0004202 A1 Jan. 3, 2013

**Related U.S. Application Data**

(63) Continuation of application No. PCT/JP2012/003747, filed on Jun. 8, 2012.

(30) **Foreign Application Priority Data**

Jun. 15, 2011 (JP) ..... 2011-133744

(51) **Int. Cl.**

*F16C 13/00* (2006.01)  
*G03G 15/02* (2006.01)  
*G03G 15/08* (2006.01)

(52) **U.S. Cl.**

CPC ..... *G03G 15/0233* (2013.01); *G03G 15/0818* (2013.01)

(58) **Field of Classification Search**

USPC ..... 492/49, 53, 54, 56  
See application file for complete search history.

(56) **References Cited**

**U.S. PATENT DOCUMENTS**

|                  |        |                          |
|------------------|--------|--------------------------|
| 7,727,134 B2     | 6/2010 | Nakamura et al.          |
| 7,798,948 B2     | 9/2010 | Kawamura et al.          |
| 7,947,339 B2     | 5/2011 | Yamauchi et al.          |
| 2012/0058300 A1* | 3/2012 | Finn et al. .... 428/141 |
| 2012/0201568 A1  | 8/2012 | Kurachi et al.           |

**FOREIGN PATENT DOCUMENTS**

|    |              |         |
|----|--------------|---------|
| EP | 1 947 526 A1 | 7/2008  |
| EP | 1 947 527 A1 | 7/2008  |
| EP | 2 128 717 A1 | 12/2009 |
| JP | 1-142749 A   | 6/1989  |
| JP | 1-257881 A   | 10/1989 |

(Continued)

**OTHER PUBLICATIONS**

International Preliminary Report on Patentability, International Application No. PCT/JP2012/003747, Mailing Date Jan. 3, 2014.

(Continued)

*Primary Examiner* — Christopher Besler

(74) *Attorney, Agent, or Firm* — Fitzpatrick, Cella, Harper and Scinto

(57) **ABSTRACT**

An electrophotographic member whose performances are hardly changed even after a long-term use is provided. An electrophotographic member having a mandrel, an elastic layer and a surface layer, wherein the surface layer contains a titanium oxide film having chemical bonds represented by the following formula (1) and formula (2) is provided.

O—Ti—O ..... Formula (1)

Ti—O—C ..... Formula (2)

**4 Claims, 3 Drawing Sheets**



(56)

**References Cited**

FOREIGN PATENT DOCUMENTS

|    |             |   |         |
|----|-------------|---|---------|
| JP | 2003-183427 | A | 7/2003  |
| JP | 2006-293004 | A | 10/2006 |
| JP | 2007-78947  | A | 3/2007  |
| JP | 2010-2567   | A | 1/2010  |
| JP | 2011-59220  | A | 3/2011  |

OTHER PUBLICATIONS

Uesugi, et al., U.S. Appl. No. 13/742,176, filed Jan. 15, 2013.  
PCT International Search Report dated Jul. 10, 2012 in International Application No. PCT/JP2012/003747.  
European Search Report dated Oct. 24, 2014 in European Application No. 12800588.1.

\* cited by examiner

*FIG. 1A**FIG. 1B*

FIG. 2



FIG. 3



FIG. 4



## 1

**ELECTROPHOTOGRAPHIC MEMBER,  
PROCESS CARTRIDGE AND  
ELECTROPHOTOGRAPHIC APPARATUS**

**CROSS-REFERENCE TO RELATED  
APPLICATIONS**

This application is a continuation of International Application No. PCT/JP2012/003747, filed Jun. 8, 2012, which claims the benefit of Japanese Patent Application No. 2011-133744, filed Jun. 15, 2011.

**BACKGROUND OF THE INVENTION**

**1. Field of the Invention**

The present invention relates to an electrophotographic member for use in a developing member, a charging member and the like, a process cartridge and an electrophotographic apparatus.

**2. Description of the Related Art**

In an electrophotographic apparatus, a developing roller is generally configured to have an elastic layer so as to ensure a sufficient nip width with respect to a photosensitive drum to thereby stably rotate. The developing roller has a surface layer formed in order to make the toner conveying ability of a surface better and suppress toner fixation on the surface.

A charging roller which is placed while being in contact with the photosensitive drum and which allows the photosensitive drum to be charged at a predetermined potential is also generally configured to have an elastic layer and a surface layer as in the developing roller.

Meanwhile, as there is an increasing demand for more improvement in durability of an electrophotographic apparatus, there is also a demand for electrophotographic members such as a developing roller and a charging roller whose changes in performance after a long-term use are smaller.

In regard to such demands, in order to improve durability of a conductive roller in the vicinity of a surface, Japanese Patent Application Laid-Open No. H01-257881 has proposed a developing roller provided with a ceramics coating layer having a thickness of 5  $\mu\text{m}$  or less on the surface of the roller. Japanese Patent Application Laid-Open No. H01-142749 has proposed a developing roller and a developer regulating member whose surfaces are coated with ceramics having titanium and tungsten atoms.

**SUMMARY OF THE INVENTION**

However, according to studies by the present inventors, the above surface layer containing ceramics has a high durability by itself, while the surface layer has a high hardness. Therefore, in the case where a conductive roller provided with such a surface layer is used as a developing roller, a so-called filming phenomenon in which a toner is fixed on the surface of the developing roller may occur.

If such filming occurs, charging performance to a toner and surface properties may be changed to thereby cause changes in the density of an electrophotographic image, and the like, before and after the occurrence of such filming. Also in the case where the conductive roller according to the above patent literatures is used as a charging roller, toner fixation on the surface may occur to thereby cause uneven charging in a photosensitive drum.

Then, the present invention is directed to providing an electrophotographic member excellent in durability, whose performances are hardly changed even after a long-term use.

## 2

Further, the present invention is directed to providing a process cartridge and an electrophotographic apparatus which can stably form a high quality electrophotographic image.

5 According to one aspect of the present invention, there is provided an electrophotographic member having a mandrel, an elastic layer and a surface layer, wherein the surface layer consists of a titanium oxide film having chemical bonds represented by the following formulae (1) and (2):



10 According to another aspect of the present invention, there is provided a process cartridge comprising the above electrophotographic member, and configured to be attachable to and removable from a main body of an electrophotographic apparatus. According to further aspect of the present invention, there is provided an electrophotographic apparatus comprising the above electrophotographic member.

15 According to the present invention, an electrophotographic member whose performances are hardly changed even after a long-term use and which is conducive to the stable formation of an electrophotographic image can be obtained.

20 According to the present invention, a process cartridge and an electrophotographic apparatus which can form a high quality electrophotographic image are provided.

25 Further features of the present invention will become apparent from the following description of exemplary embodiments with reference to the attached drawings.

**BRIEF DESCRIPTION OF THE DRAWINGS**

30 FIG. 1A is a cross-sectional schematic view of a roller-shaped electrophotographic member (electrophotographic conductive roller) according to the present invention.

35 FIG. 1B is a cross-sectional schematic view of a roller-shaped electrophotographic member (electrophotographic conductive roller) according to the present invention.

40 FIG. 2 is a schematic view of one example of an electrophotographic apparatus according to the present invention.

45 FIG. 3 is a schematic view of one example of a developing apparatus according to the present invention.

FIG. 4 is an illustrative view relating to a CVD apparatus which can be used for forming a surface layer according to the present invention.

**DESCRIPTION OF THE EMBODIMENTS**

50 Preferred embodiments of the present invention will now be described in detail in accordance with the accompanying drawings.

An electrophotographic member according to the present invention is used for a developing roller, a charging roller and the like in an electrophotographic apparatus. FIGS. 1A and 1B each illustrate a cross-sectional schematic view of one example of a conductive roller of the present invention. FIGS. 1A and 1B are cross-sectional schematic views in cutting the conductive roller parallel and perpendicular to the axial direction of a mandrel, respectively. The conductive roller has an elastic layer 1b on the outer periphery of a mandrel 1a, and a surface layer 1c on the outer periphery of the elastic layer 1b. (Mandrel)

55 Any mandrel can be applied to the present invention as long as the mandrel serves as an electrode of a conductive member and a supporting member. As materials for such a mandrel, for example, metals or alloys, such as aluminum, copper, stain-

less steel and iron, and conductive materials such as conductive synthetic resins can be used.

(Elastic Layer)

The elastic layer can be a layer for allowing the conductive roller to have elasticity, in order for the roller to be brought into contact with a photosensitive drum or a developer regulating member while having an appropriate area at the time of pressure-contact with the photosensitive drum or the developer regulating member. Unless deviating from such an object, the elastic layer can be a single layer or a multilayer.

The elastic layer for use in the present invention can be prepared using any known material in a conductive roller for an electrophotographic apparatus, and for example, the following rubbers and conducting agents can be used as the material.

Examples of the rubber include ethylene-propylene-diene copolymer rubbers (EPDM), acrylonitrile-butadiene rubbers (NBR), chloroprene rubbers (CR), natural rubbers (NR), isoprene rubbers (IR), styrene-butadiene rubbers (SBR), fluororubbers, silicone rubbers, epichlorohydrin rubbers, butadiene rubbers (BR), hydrogenated products of NBR, polysulfide rubbers and urethane rubbers. It is to be noted that one kind or a mixture of several kinds of the above rubbers can also be used for the elastic layer.

As the conducting agent compounded in the elastic layer, for example, carbon black can be used, and there is no limitations on carbon black which can be used. Examples include acetylene blacks high in conductivity and furnace blacks such as SAF, ISAF, HAF, MAF, FEF, GPF and SRF. Herein, the resistance of the conductive roller can be  $1.0 \times 10^2$  to  $1.0 \times 10^{12}$ , and thus the amount of carbon black added is preferably 1 part by mass or more and 80 parts by mass or less, and more preferably in a range of 2 parts by mass or more and 70 parts by mass or less, based on 100 parts by mass of the rubber.

Other conducting agent can be used in combination with carbon black, if necessary. Examples include various conductive metals or alloys, such as graphite, aluminum, copper, tin and stainless steel, and metal oxides obtained by subjecting tin oxide, zinc oxide, indium oxide, titanium oxide, tin oxide-antimony oxide solid solution, and the like to respective conducting treatments. Herein, the resistance of the conductive roller can be  $1.0 \times 10^2$  to  $1.0 \times 10^{12}$ , and thus the amount of the other conducting agent added is preferably 2 parts by mass or more and 20 parts by mass or less, and more preferably in a range of 5 parts by mass or more and 18 parts by mass or less, based on 100 parts by mass of the rubber.

As other various additives, any known additives in the conductive roller for an electrophotographic apparatus can be used. For example, a reinforcing agent and a heat transfer improving agent, such as hydrophilic silica, hydrophobic silica, quartz, calcium carbonate, aluminum oxide, zinc oxide and titanium oxide, can also be added if necessary.

As a production method for providing the elastic layer on the mandrel, any known method in an electrophotographic conductive roller can be used. Examples include a method of extruding the mandrel and the material for the elastic layer together for molding, and a method in which, when the material for forming the elastic layer is liquid, the material is poured into a mold provided with a cylindrical pipe, holding members provided on both ends of the pipe, for holding the mandrel, and the mandrel, and heated and cured.

The elastic layer can also be a single layer or a multilayer as described above. For example, for the purpose of providing asperity on the periphery of a first elastic layer formed by using the rubber and the conducting agent, a second elastic layer can be provided.

In the case where a rubber layer having a thickness of several  $\mu\text{m}$  to several mm is provided as the second elastic layer, the rubber layer can be provided using a material for forming the second elastic layer by any known method in the electrophotographic roller. In the case where a resin layer is provided as the second elastic layer, any known resin can be used as the material. Specific examples include fluorine resins, polyamide resins, acrylic urethane resins, phenol resins, melamine resins, silicone resins, urethane resins, polyester resins, polyvinyl acetal resins, epoxy resins, polyether resins, amino resins, acrylic resins, urea resins and mixtures of these resins.

When the resin layer is provided as the second elastic layer, a resin having carbon black added thereto can be used. Examples include carbon black having a high conductivity, such as EC300J and EC600JD (both are trade names, produced by Lion Corporation), and carbon black for rubbers or carbon black for coating materials, having a moderate conductivity. Carbon black for coating materials can be used from the viewpoint of control of dispersibility and conductivity. Since the conductive roller can have a moderate resistance, the amount of carbon black compounded can be 3 parts by mass or more and 30 parts by mass or less based on 100 parts by mass of a resin component.

As a method for providing a resin layer having a thickness of several  $\mu\text{m}$  to several tens  $\mu\text{m}$  as the second elastic layer, for example, there is a method in which the resin layer is obtained by mixing and dispersing the resin component and carbon black with and in a solvent to form a coating liquid, and coating the coating liquid on the first elastic layer.

As the solvent for use in the coating liquid, a solvent can be appropriately used as long as the solvent dissolves the resin for use in the resin layer. Examples include ketones such as methyl ethyl ketone and methyl isobutyl ketone, hydrocarbons such as hexane and toluene, alcohols such as methanol and isopropanol, esters and water. Methyl ethyl ketone and methyl isobutyl ketone can be particularly used from the viewpoints of solubility of the resin and boiling point.

(Surface Layer)

The surface layer contains a titanium oxide film having chemical bonds represented by the following formula (1) and formula (2), respectively.



Namely, in the titanium oxide film according to the present invention, at least one portion of titanium atoms forming the titanium oxide film is bound to carbon atoms via oxygen atoms. The titanium oxide film having such a configuration enables providing high flexibility for the titanium oxide film and high adhesiveness for the elastic layer. Herein, the respective chemical bonds of the formula (1) and the formula (2) in the surface layer can be identified by using a scanning phototransistor.

The amount of the bond represented by the formula (2) in the titanium oxide film can be 20% or more and 80% or less based on the total number of Ti atoms of the formula 1 and the formula 2 in terms of the number of Ti atoms. Such a range enables providing for the surface layer high durability and sufficient elasticity for suppressing the filming of a toner.

A conventional conductive roller in which a titanium oxide film containing only the bond represented by the formula (1) is formed on an elastic layer as a surface layer has caused the filming of a toner in some cases because the hardness of the surface layer is high and the smoothness of the surface is low.

On the other hand, since at least one portion of titanium atoms forming the titanium oxide film is bound to carbon atoms via oxygen atoms in the present invention, the density of the titanium oxide film is reduced on some level. Therefore, it is considered that, as compared with the conventional titanium oxide film, the titanium oxide film of the present invention is rich in flexibility and excellent in conformability to deformation of the elastic layer, and peeling off of the surface layer from the elastic layer during use is suppressed.

The titanium oxide film according to the present invention can have a surface resistance of  $1.0 \times 10^7 \Omega/\square$  or more and  $1.0 \times 10^{11} \Omega/\square$  or less. Therefore, the surface layer according to the present invention is resistant to electrostatic adhesion to a toner as compared with a surface layer containing insulating ceramics. Herein, the surface layer having conductivity means that the surface resistance of the surface layer is  $1 \times 10^3 \Omega/\square$  or more and  $1 \times 10^{13} \Omega/\square$  or less. In addition, the surface layer having insulating properties means that the surface resistance of the surface layer is more than  $1 \times 10^{13} \Omega/\square$ . The surface resistance of the titanium oxide film (surface layer) can be specified by forming a film on a polyester film and measuring the surface resistance of the formed film by using an ultrahigh resistance/microammeter: R8340 (trade name, Advantest Corporation).

The thickness of the surface layer is preferably 5 nm or more and 1  $\mu\text{m}$  or less, and particularly preferably 10 nm or more and 0.9  $\mu\text{m}$  or less, from the viewpoints of intensity and flexibility as the surface layer.

<Production Method of Titanium Oxide Film>

The titanium oxide film according to the present invention can be formed by, for example, a physical vapor deposition (PVD) method such as vacuum vapor deposition and ion plating, a chemical vapor deposition (CVD) method such as plasma CVD, thermal CVD and laser CVD, or a sol-gel method.

In the case where a titanium oxide film containing titanium atoms bound to alkyl groups via oxygen atoms (hereinafter, referred to also as an "alkoxy-modified titanium oxide film") is produced by, for example, a plasma CVD method, the titanium oxide film can be formed by, for example, the following apparatus and procedure. Namely, such an apparatus has, as illustrated in FIG. 4, a vacuum chamber 41, two plate electrodes 42 placed in parallel, a raw material gas cylinder and a raw material liquid tank 43, a raw material supply unit 44, a unit 45 for exhausting the gas in the chamber, a high-frequency supply power source 46 for supplying a high-frequency wave, and a motor 47 for rotating an elastic roller 48.

Procedure (1)

Place the elastic roller 48 having an elastic layer formed on a mandrel between the two plate electrodes 42, and rotate the mandrel around the axis by driving the motor 47 so that the alkoxy-modified titanium oxide film is uniformly formed.

Procedure (2)

Evacuate the inside of the vacuum chamber 41 until reaching, specifically, for example, 2 Pa or less, preferably, 1 Pa or less, by the exhaust unit.

Procedure (3)

Introduce a raw material gas through a raw material introduction port, confirm that the inside of the vacuum chamber 41 reaches the constant pressure, and thereafter supply a high-frequency power to the plate electrodes 42 by the high-frequency supply power source 46 to generate plasma for forming a film.

Procedure (4)

After a lapse of a predetermined period, stop the supply of the raw material gas and the high-frequency power, introduce (leak) air or nitrogen into the vacuum chamber 41 until reach-

ing atmospheric pressure, and take out the elastic roller having the alkoxy-modified titanium oxide film formed on the surface of the roller.

According to the procedures as described above, the conductive roller having the alkoxy-modified titanium oxide film can be produced. It is to be noted that many elastic rollers 48 may be simultaneously treated by plasma CVD as long as the rollers are placed under a uniform plasma atmosphere.

Herein, gaseous or gasified titanium tetraalkoxide is usually used as the raw material gas, and, if necessary, the titanium tetraalkoxide is introduced together with an inert gas such as argon or helium or an oxidizing gas.

Examples of the titanium tetraalkoxide include a compound represented by the following formula (3).



In the formula (3), R represents a linear or branched-chain alkyl group having 2 to 18 carbon atoms.

Specific examples include the following: titanium tetraethoxide, titanium tetraisopropoxide, titanium tetra-n-butoxide, titanium tetra-tert-butoxide and titanium tetra-2-ethyl hexoxide.

The titanium tetraalkoxides can be used singly or as a mixture of a plurality of the titanium tetraalkoxides.

The alkoxy-modified titanium oxide film according to the present invention can also be produced by controlled hydrolysis and condensation of the titanium tetraalkoxide. Namely, the alkoxy-modified titanium oxide film according to the present invention can contain the hydrolytic condensate of the titanium tetraalkoxide. One specific example of such a production method includes a sol-gel method.

In the sol-gel method, the titanium tetraalkoxide is first added to a mixed solvent of an alcohol and water. The mixing ratio of an alcohol and water can be set without any limitation as long as the titanium tetraalkoxide is dissolved. As such an alcohol, alcohols soluble in water, such as methanol, ethanol, isopropyl alcohol and tert-butyl alcohol, can be arbitrarily used.

Thereafter, in order to modulate viscosity and improve 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350

surface of the developing roller due to excessive charging of a toner can be suppressed with more certainty.

Herein, the surface potential of the conductive roller can be measured by the following method. Namely, the surface potential can be determined by using a dielectric relaxation analysis system of a semi-insulating device, manufactured by Quality Engineering Associates, Inc., to measure surface potentials in respective points obtained by dividing the conductive roller into 260 in the longitudinal direction and into 18 in the circumferential direction, and calculating the mean value of the surface potentials.

From the viewpoint of optimizing the elastic modulus of the titanium oxide film according to the present invention, an abundance ratio ( $C_{C-C}/O_{C-O}$ ) of an abundance ratio of an oxygen atom bound to a carbon atom, ( $O_{C-O}$ ), to a carbon atom bound to a carbon atom, ( $C_{C-C}$ ), is preferably 3 or more and 8 or less, and particularly preferably 3 or more and 6 or less.

It is to be noted that the proportion ( $C_{C-C}/O_{C-O}$ ) of the abundance ratio of an oxygen atom bound to a carbon atom to the abundance ratio of a carbon atom bound to a carbon atom can be calculated by measuring the abundance ratio ( $O_{C-O}$ ) of an oxygen atom of a carbon atom-oxygen atom bond and the abundance ratio ( $C_{C-C}$ ) of a carbon atom of a carbon atom-carbon atom bond in terms of amount by using a scanning X-ray photoelectron spectrometer, and determining the proportion of both the abundance ratios. As an analyzing apparatus in this case, PHI 5000 VersaProbe (trade name, ULVAC-PHI, Incorporated) can be used.

(Electrophotographic Apparatus and Developing Apparatus)

One example of an electrophotographic apparatus for which the conductive roller of the present invention can be used is illustrated in FIG. 2. It is to be noted that in this example, the conductive roller of the present invention is used as a developing roller. A color electrophotographic apparatus illustrated in the schematic view of FIG. 2 has developing apparatuses (for each color) (10a to 10d) in a tandem form, which are provided for respective color toners of yellow Y, magenta M, cyan C and black BK.

The developing apparatuses, whose specifications are slightly different from one another depending on properties of respective color toners, basically have the same structure. Each developing apparatus is provided with a photosensitive drum 2 which rotates in the arrow direction. A charging roller 9 for uniformly charging the photosensitive drum 2, a light exposure unit for irradiating the uniformly charged photosensitive drum 2 with laser light 21 to form an electrostatic latent image, and a hopper 3 for supplying a toner to the photosensitive drum 2, on which the electrostatic latent image is formed, to develop the electrostatic latent image are provided around the developing apparatus. Furthermore, a transfer member is provided which has a transfer roller 26 for transferring a toner image on the photosensitive member 2 onto a recording medium (transfer material) 24 such as paper which is fed by a paper-feeding roller 22 and conveyed by a conveying belt 23, while a voltage from a bias power source 25 is applied from the back surface of the recording medium 24.

The conveying belt 23 is suspended on a driving roller 27, a driven roller 28 and a tension roller 29, and is controlled so as to move in synchronization with image-forming portions and convey the recording medium 24 so that the toner images formed in the respective image-forming portions are sequentially superimposed and transferred onto the recording medium 24. It is to be noted that the recording medium 24 is electrostatically adsorbed to the conveying belt 23 by the

operation of an adsorption roller 30 provided right before the conveying belt 23, and is to be conveyed.

In the electrophotographic apparatus, the photosensitive drum 2 and the developing roller which is a conductive roller 1 of the present invention are placed so as to be in contact with each other, and rotate in the same direction at a position at which the photosensitive drum 2 is in contact with the developing roller. The electrophotographic apparatus is further provided with a fixing apparatus 31 for fixing the toner images which are superimposed and transferred onto the recording medium 24 by heating and the like, and a conveying apparatus (not illustrated) for discharging the image-formed recording medium to the outside of the apparatus. It is to be noted that the recording medium 24 is peeled from the conveying belt 23 by the operation of a peeling apparatus 32 and is to be sent to the fixing apparatus 31. On the other hand, the developing apparatus is provided with a cleaning member having a cleaning blade 33 for removing the transfer residual toner which is not transferred onto the photoreceptor 2 and remains, and a waste toner container 34 for storing the toner scraped off from the photoreceptor. The cleaned photosensitive drum 2 stands ready in the state of capable of forming an image.

Next, FIG. 3 illustrates one example of a developing apparatus. In the developing apparatus, a photosensitive drum 2 as an electrostatic latent image support member for supporting an electrostatic latent image formed by any known process is rotated in the arrow B direction. A stirring blade 5 for stirring an one-component non-magnetic toner 4 is provided in a hopper 3 which is a toner container. The toner 4 is supplied to a developing roller which is the conductive roller 1 of the present invention, which a toner-supplying member 6 for peeling off the toner 4 existing on the surface of the developing roller after developing abuts. A supply roller which is the toner-supplying member rotates in the same direction (arrow C direction) as the direction (arrow A direction) of the developing roller, and thus the surface of a toner-supplying/peeling off roller moves in the direction counter to the surface of the developing roller. Therefore, an one-component non-magnetic toner having a non-magnetic toner supplied from the hopper 3 is supplied to the developing roller. A developing bias voltage is applied to the developing roller from a developing bias power source 7 in order to allow the one-component non-magnetic toner 4 having a non-magnetic toner supplied on the developing roller to move.

The toner-supplying/peeling off member 6 can be an elastic roller member of resin, rubber, sponge or the like. Once the toner-supplying/peeling off member 6 peels off the toner, which is not developed and transferred to the photosensitive drum 2, from the surface of the developing roller, then generation of the unmoving toner on the developing roller is inhibited to thereby allow a toner to be uniformly charged.

As a member for regulating the layer thickness of the one-component non-magnetic toner 4 on the developing roller, a toner regulating member 8 made of a material having rubber elasticity, such as a urethane rubber or a silicone rubber, or a material having metal elasticity, such as phosphor bronze or stainless copper can be used. The toner regulating member 8 is brought into pressure-contact with the developing roller in the opposite direction to the rotational direction of the developing roller, thereby enabling forming a much thinner toner layer on the developing roller.

The process cartridge of the present invention can be provided with the electrophotographic member of the present invention as, for example, a charging roller, and can be configured to be attachable to and removable from the main body of the electrophotographic apparatus.

**9**  
EXAMPLES

Hereinafter, the present invention will be described in more detail with reference to Examples.

[Shape of Conductive Roller]

In each Example, a conductive roller was produced so as to allow the shape of the conductive roller to be the following diameter of a cored bar and the following thickness of an elastic layer depending on each application. Herein, in the case where an elastic layer had a two-layer structure, the sum of the two layers was made to have the following thickness.

Developing roller: diameter of cored bar=6 mm, thickness of elastic layer=3.0 mm

Charging roller: diameter of cored bar=6 mm, thickness of elastic layer=1.25 mm

With respect to a second elastic layer and a surface layer, an elastic layer and a surface layer each having the described thickness were produced in both cases of the developing roller and the charging roller.

[Production of Elastic Roller]

First, the following elastic rollers each having a mandrel (cored bar) and an elastic layer were prepared.

Preparation of Elastic Roller 1-1

A conductive mandrel made of stainless steel (SUS304) was used for a cored bar. A silane coupling primer (trade name: DY35-051, Dow Corning Toray Co., Ltd.) was applied onto the periphery of the mandrel, and then baked at a temperature of 150° C. for 60 minutes.

Then, the mandrel was coaxially placed on the inside of a cylindrical mold, and the space between the inner periphery of the mold and the periphery of the mandrel was filled with a liquid material for forming an elastic layer, in which materials shown in the following Table 1 were dispersed, followed by heating at a temperature of 150° C. for 20 minutes. After cooling, the mandrel was released from the mold, and heated in an oven heated at a temperature of 200° C. for 5 hours, thereby providing a first elastic layer around the mandrel.

TABLE 1

| Material for forming first elastic layer                                             | Parts by mass |
|--------------------------------------------------------------------------------------|---------------|
| Silicone rubber: XE15-645A liquid (trade name, Momentive Performance Materials Inc.) | 50            |
| Silicone rubber: XE15-645B liquid (trade name, Momentive Performance Materials Inc.) | 50            |
| Carbon black: HS-100 (trade name, Denki Kagaku Kogyo Kabushiki Kaisha)               | 10            |

Then, a second elastic layer (resin layer) was provided on the periphery of the first elastic layer as follows. Namely, materials shown in Table 2 were added to methyl ethyl ketone (MEK) and well mixed, and the obtained mixture was charged into an overflow-type circulation coating apparatus. The mandrel provided with the first elastic layer was dipped in the circulation coating apparatus, pulled up and then air-dried for 30 minutes, and thereafter heated in an oven heated to a temperature of 150° C. for 5 hours to provide a second elastic layer having a thickness of 20 µm, thereby producing an elastic roller 1-1 having a mandrel and an elastic layer having a two-layer structure.

**10**  
TABLE 2

| Material for forming second elastic layer                                              | Parts by mass |
|----------------------------------------------------------------------------------------|---------------|
| Polyl: N5120 (trade name, Nippon Polyurethane Industry Co., Ltd.)                      | 87            |
| Isocyanate: L-55E (trade name, Nippon Polyurethane Industry Co., Ltd.)                 | 13            |
| Carbon black: MA77 (trade name, Mitsubishi Chemical Corporation)                       | 35            |
| Acrylic particle: G-400 transparent (trade name, Negami Chemical Industrial Co., Ltd.) | 10            |

Preparation of Elastic Rollers 1-2 to 1-6

Elastic rollers 1-2 to 1-6 were prepared in the same manner as the elastic roller 1-1 except that the amounts of the carbon black were changed to 12 parts by mass, 15 parts by mass, 8 parts by mass, 18 parts by mass, and 13 parts by mass in Table 1.

Preparation of Elastic Roller 2-1

A silane coupling primer: DY35-051 (trade name, Dow Corning Toray Co., Ltd.) was applied to a mandrel made of stainless steel: SUS304, and then baked at a temperature of 150° C. for minutes. Then, a rubber mixture obtained by well kneading materials shown in the following Table 3 was provided on the mandrel by a crosshead extruder, and heated at a temperature of 170° C. for 20 minutes, thereby preparing an elastic roller 2-1.

TABLE 3

| Material for forming first elastic layer                                      | Parts by mass |
|-------------------------------------------------------------------------------|---------------|
| Silicone rubber: TSE270-5U (trade name, Momentive Performance Materials Inc.) | 92            |
| Crosslinking agent: TC-8 (trade name, Momentive Performance Materials Inc.)   | 8             |
| Carbon black: Denka Black (trade name, Denki Kagaku Kogyo Kabushiki Kaisha)   | 10            |

Preparation of Elastic Rollers 2-2 to 2-3

Elastic rollers 2-2 to 2-3 were prepared in the same manner as in the elastic roller 2-1 except that the amounts of the carbon black compounded were changed to 15 parts by mass and 50 parts by mass in Table 3.

Preparation of Elastic Roller 3-1

A primer: Metaloc U-20 (trade name, Toyokagaku Kenkyusho Co., Ltd.) was applied to a mandrel made of stainless steel: SUS304, dried at a temperature of 80° C. for 30 minutes, and then further heated at 120° C. for 60 minutes. Then, a rubber mixture obtained by well kneading materials shown in the following Table 4 was provided on the mandrel by a crosshead extruder, and heated at a temperature of 150° C. for 50 minutes, thereby preparing an elastic roller 3-1.

## 11

TABLE 4

| Material for forming first elastic layer                                                                     | Parts by mass |
|--------------------------------------------------------------------------------------------------------------|---------------|
| Acrylonitrile butadiene rubber: JSR N231L (trade name, JSR Corporation)                                      | 100           |
| Zinc oxide: two kinds of zinc oxides (HakusuiTech Co., Ltd.)                                                 | 5             |
| Stearic acid: Stearic acid S (trade name, Kao Corporation)                                                   | 2             |
| Sulfur: dispersible sulfur: Sulfax 200S (trade name, produced by Tsuruimi chemical Industry Co., Ltd.)       | 1.2           |
| Di-2-benzothiazolyl tetrasulfide: Nocceler DM (trade name, Ouchi Shinko Chemical Industrial Co., Ltd.)       | 1.0           |
| Dipentamethylene thiuram tetrasulfide: Nocceler TRA (trade name, Ouchi Shinko Chemical Industrial Co., Ltd.) | 1.0           |
| Tetramethyl thiuram monosulfide: Nocceler TS (trade name, Ouchi Shinko Chemical Industrial Co., Ltd.)        | 1.0           |
| Plasticizer: Polycizer W-1600 (trade name, DIC Corporation)                                                  | 50            |
| Carbon black: Toka Black #7360SB (trade name, Tokai Carbon Co., Ltd.)                                        | 40            |

## Preparation of Elastic Rollers 3-2 to 3-3

Elastic rollers 3-2 to 3-3 were prepared in the same manner as in the elastic roller 3-1 except that the amounts of the carbon black compounded were changed to 30 parts by mass and 50 parts by mass in Table 4.

## Preparation of Elastic Roller 4-1

A primer: Metaloc U-20 (trade name, Toyokagaku Kenkyusho Co., Ltd.) was applied to a mandrel made of stainless steel: SUS304, dried at a temperature of 80°C. for 30 minutes, and then further heated at 120°C. for 60 minutes. Then, a rubber mixture obtained by well kneading materials shown in the following Table 5 was provided on the mandrel by a crosshead extruder, and heated at a temperature of 140°C. for 60 minutes, thereby preparing an elastic roller 4-1.

TABLE 5

| Material for forming first elastic layer                                                                     | Parts by mass |
|--------------------------------------------------------------------------------------------------------------|---------------|
| Epichlorohydrin-ethylene oxide-allyl glycidyl ether terpolymer: Epicholomer CG (trade name, Daiso Co., Ltd.) | 100           |
| Stearic acid: Stearic acid S (trade name, produced by Kao Corporation)                                       | 2             |
| Calcium carbonate: Nanox #30 (trade name, Maruo Calcium Co., Ltd.)                                           | 45            |
| Carbon black: Toka Black #7360SB (trade name, Tokai Carbon Co., Ltd.)                                        | 5             |
| Sulfur: dispersible sulfur: Sulfax 200S (trade name, produced by Tsuruimi Chemical Industry Co., Ltd.)       | 1.2           |
| Di-2-benzothiazolyl tetrasulfide: Nocceler DM (trade name, Ouchi Shinko Chemical Industrial Co., Ltd.)       | 1.0           |
| Dipentamethylene thiuram tetrasulfide: Nocceler TRA (trade name, Ouchi Shinko Chemical Industrial Co., Ltd.) | 1.0           |

## Preparation of Elastic Rollers 4-2 to 4-3

Elastic rollers 4-2 to 4-3 were prepared in the same manner as in the elastic roller 4-1 except that the amounts of the carbon black compounded were changed to 8 parts by mass and 1 part by mass in Table 5.

## Preparation of Elastic Roller 5

A second elastic layer was provided on the periphery of the elastic roller 2-1 as follows. Namely, materials shown in Table 6 were weighed and methyl isobutyl ketone (MIBK)

## 12

was added thereto, and the well-stirred mixture was charged into an overflow-type circulation coating apparatus. The elastic roller 2 was dipped in the coating apparatus, pulled up and then heated at a temperature of 80°C. for 1 hour, and thereafter further heated at a temperature of 160°C. for 1 hour to provide a second elastic layer having a thickness of 20 µm, thereby producing an elastic roller 5.

TABLE 6

| Material for forming second elastic layer                                  | Parts by mass |
|----------------------------------------------------------------------------|---------------|
| Acrylic polyol: Placel DC2016 (trade name, Daicel Corporation)             | 55.5          |
| 15 Isocyanate 1: Duranate TPA-B80E (trade name, Asahi Kasei Corporation)   | 31.2          |
| Isocyanate 2: Vestanat B1370 (trade name, Degussa-Huls AG)                 | 13.3          |
| Titanium oxide: MTY02 (trade name, Tayca Corporation)                      | 11.1          |
| Carbon black: MA11 (trade name, Mitsubishi Chemical Corporation)           | 25.0          |
| 20 Dimethylsilicone oil: SH28PA (trade name, Dow Corning Toray Co., Ltd.)  | 0.04          |
| Polymethylmethacrylate resin particle: C-12 (trade name, Toyobo Co., Ltd.) | 5.5           |

## (Elastic Roller 6)

The second elastic layer according to the elastic roller 5 was provided on the periphery of the elastic roller 3-1. This is referred to as an elastic roller 6.

## (Elastic Roller 7)

The second elastic layer according to the elastic roller 5 was provided on the periphery of the elastic roller 4-1. This is referred to as an elastic roller 7.

## Example 1

## Preparation of Electrophotographic Roller 1-1

According to the following method, a surface layer was formed on the periphery of the elastic layer of the prepared elastic roller 1-1 as described above. Namely, the elastic roller 1-1 was set in a CVD apparatus illustrated in FIG. 4, and the inside of a chamber was evacuated until reaching 2 Pa by a vacuum pump. Then, while gasified titanium tetraisopropoxide was introduced into the chamber at a flow rate of 5 cm<sup>3</sup>/sec and the elastic roller 1-1 was rotated at a rotation number of 20 rpm, a 70 W of power at a frequency of 13.56 MHz was supplied between plate electrodes by a high-frequency power source to generate plasma between the electrodes. Such a state was maintained for 120 seconds to thereby produce a surface layer having a thickness of 100 nm on the periphery of the elastic roller 1-1. Thus, an electrophotographic roller 1-1 was prepared.

## Examples 1-2 to 1-3

## Preparation of Electrophotographic Rollers 1-2 to 1-3

Electrophotographic rollers 1-2 to 1-3 were prepared in the same manner as in the electrophotographic roller 1-1 except that the elastic roller 1-1 was changed to the elastic roller 1-2 or the elastic roller 1-3.

[Evaluation (1): Confirmation of Presence of Chemical Bonds Represented by Formula 1 and Formula 2]

The surface layer of each of the electrophotographic rollers 1-1 to 1-3 according to Example 1 was analyzed by using a scanning X-ray photoelectron spectrometer (trade name: PHI

5000 VersaProbe, ULVAC-PHI, Incorporated), and the presences of an O—Ti—O bond and a Ti—O—C bond were confirmed.

[Evaluation (2): Evaluation of Oxygen-Carbon Atom Ratio  $C_{C-C}/O_{C-O}$ ]

With respect to the surface layer of each of the electrophotographic rollers 1-1 to 1-3 according to Example 1, the abundance ratio ( $C_{C-C}$ ) of a carbon atom bound to a carbon atom and the abundance ratio ( $O_{C-O}$ ) of an oxygen atom bound to a carbon atom were measured in terms of amount by using a scanning X-ray photoelectron spectrometer (trade name: PHI 5000 VersaProbe, ULVAC-PHI, Incorporated) to determine the proportion ( $C_{C-C}/O_{C-O}$ ).

[Evaluation (3): Surface Resistance of Titanium Oxide Film Forming Surface Layer]

A titanium oxide film was formed on a polyester film by using the same method as in the surface layer according to Example 1, and the surface resistance of the titanium oxide film was measured by using an ultrahigh resistance/microammeter (trade name: R8340, Advantest Corporation) when an applied voltage was 300 V.

[Evaluation (4): Evaluation of Surface Potential]

With respect to each of the electrophotographic rollers 1-1 to 1-3 according to Example 1, surface potentials were measured in respective points obtained by dividing each roller into 260 in the longitudinal direction and into 18 in the circumferential direction. The arithmetic mean value of the surface potentials at all points measured was defined as the surface potential of each electrophotographic roller,  $V_p$ .

Then, the surface of each electrophotographic roller after  $V_p$  had been measured was cut out by a polishing machine by a thickness of 10  $\mu\text{m}$  in the depth direction from the surface. The surface potentials of each electrophotographic roller after polishing were measured to calculate the mean value, as described above, thereby obtaining the surface potential,  $V_e$ , of each electrophotographic roller after polishing. The  $V_p/V_e$  was determined from the surface potentials  $V_p$  and  $V_e$ . Herein, the surface potentials were measured by using a dielectric relaxation analysis system manufactured by Quality Engineering Associates, Inc.

[Evaluation (5): Evaluation for Use as Developing Roller (I)]

<Evaluation (5)-1>: Evaluation of Ghost Performance

Each of the electrophotographic rollers 1-1 to 1-3 according to Example 1 was mounted as a developing roller to a process cartridge for a color laser printer (trade name: LBP7700C (altered machine), manufactured by Canon Inc.). The process cartridge was loaded to the color laser printer, and 20,000 sheets of electrophotographic images were output under an environment of a temperature of 30°C. and a relative humidity of 80% and under an environment of a temperature 15°C. and a relative humidity of 10%. The electrophotographic images were images in which 4-point size letters of alphabet "E" were printed on an A4-size sheet so that the printing percentage was 1%. Subsequently, the following image was output.

Image for Evaluating Ghost Performance

A total of 2 sheets each having a different image pattern from each other were used, in which each image pattern had six solid images having a square of 20 mm on a side and arranged next to each other on the upper portion of a sheet of paper as well as a halftone pattern located below the upper portion over the whole area, and one image pattern had a halftone density different from a halftone density of the other image pattern. Herein, one halftone used had a density of 0.4 and the other had a density of 0.7 as measured by a spectral densitometer: X-Rite 504 (trade name, S.D.G K.K.).

The obtained images were visually observed and evaluated according to the criteria in the following Table 7.

TABLE 7

| Rank | Criteria                                                                                                   |
|------|------------------------------------------------------------------------------------------------------------|
| A    | No uneven density in a square of 20 mm on a side was observable on halftones of both image patterns.       |
| B    | Uneven density in a square of 20 mm on a side was slightly observable on a halftone of one image pattern.  |
| C    | Uneven density in a square of 20 mm on a side was slightly observable on halftones of both image patterns. |

<Evaluation (5)-2>: Filming Evaluation

15 The electrophotographic roller which had been used as the developing roller was taken out from the process cartridge, and the surface of the electrophotographic roller was observed by an optical microscope and evaluated according to the criteria described in the following Table 8.

TABLE 8

| Rank | Criteria                      |
|------|-------------------------------|
| A    | No toner was adhered.         |
| B    | Toner was slightly fixed.     |
| C    | Toner was considerably fixed. |

[Evaluation (6): Evaluation for Use as Developing Roller (II)]

<Evaluation (6)-1>

35 Each of the electrophotographic rollers 1-1 to 1-3 according to Example 1 was mounted as a developing roller to a process cartridge for a color laser printer (trade name: LBP7700C (altered machine), manufactured by Canon Inc.). The process cartridge was loaded to the color laser printer, and 20,000 sheets of electrophotographic images were output under an environment of a temperature of 30°C. and a relative 40 humidity of 80%. The electrophotographic images were images in which 4-point size letters of alphabet "E" were printed on an A4-size sheet so that the printing percentage was 1%. Subsequently, a solid white image was output, and then a reflection density was measured by a white photometer 45 TC-60DS/A (trade name, Tokyo Denshoku Co., Ltd.). Herein, the difference between reflection densities of a not-printed area before and after printing was defined as fogging (%) and evaluated according to the criteria described in the 50 following Table 9.

TABLE 9

| Rank | Criteria                                   |
|------|--------------------------------------------|
| A    | Fogging was less than 1.0%.                |
| B    | Fogging was 1.0% or more and 3.0% or less. |
| C    | Fogging was more than 3.0%.                |

<Evaluation (6)-2>

60 After the solid white image subjected to the evaluation of Evaluation (6)-1 was output, the electrophotographic roller which had been used as the developing roller was taken out from the process cartridge, and the presence and degree of 65 scraping on the surface were observed by an optical microscope and evaluated according to the criteria described in the following Table 10.

## 15

TABLE 10

| Rank | Criteria                                         |
|------|--------------------------------------------------|
| A    | No scraping was observed on the surface.         |
| B    | Scraping was slightly observed on the surface.   |
| C    | Scraping was observed on the surface.            |
| D    | Scraping was remarkably observed on the surface. |

## Example 2

## Preparation of Electrophotographic Rollers 2-1 to 2-3

Electrophotographic rollers 2-1 to 2-3 were prepared in the same manner as in the electrophotographic rollers 1-1 to 1-3 according to Example 1 except that titanium tetra-n-butoxide was used as a raw material gas, and subjected to Evaluations (1) to (6).

## Example 3

## Preparation of Electrophotographic Rollers 3-1 to 3-3

Electrophotographic rollers 3-1 to 3-3 were prepared in the same manner as in the electrophotographic rollers 1-1 to 1-3 according to Example 1 except that a mixture of titanium tetra-n-butoxide and titanium tetra-2-ethyl hexoxide (=1/1, in molar ratio of Ti atoms) was used as a raw material gas, and subjected to Evaluations (1) to (6).

## Example 4

Electrophotographic rollers 4-1 to 4-3 were prepared in the same manner as in the electrophotographic rollers 1-1 to 1-3 according to Example 1 except that titanium tetra-2-ethyl hexoxide was used as a raw material gas, and subjected to Evaluations (1) to (6).

## Example 5

Electrophotographic rollers 5-1 to 5-3 were prepared in the same manner as in the electrophotographic rollers 1-1 to 1-3 according to Example 1 except that titanium tetraethoxide was used as a raw material gas, and subjected to Evaluations (1) to (6).

## Example 6

## Preparation of Electrophotographic Rollers 6-1 to 6-2

Electrophotographic rollers 6-1 to 6-2 were prepared in the same manner as in the electrophotographic roller 1-1 according to Example 1 except that the elastic rollers 1-4 and 1-5 were used, and subjected to Evaluations (1) to (6).

## Example 7

## Preparation of Electrophotographic Rollers 7-1 to 7-2

Electrophotographic rollers 7-1 to 7-2 were prepared in the same manner as in the electrophotographic rollers 6-1 to 6-2

## 16

according to Example 6 except that a mixture of titanium tetra-n-butoxide and titanium tetra-2-ethyl hexoxide (=1/1, in molar ratio of Ti atoms) was used as a raw material gas, and subjected to Evaluations (1) to (6).

## Example 8

## Preparation of Electrophotographic Rollers 8-1 to 8-2

10 Electrophotographic rollers 8-1 to 8-2 were prepared in the same manner as in the electrophotographic rollers 6-1 to 6-2 according to Example 6 except that titanium tetra-2-ethyl hexoxide was used as a raw material gas, and subjected to Evaluations (1) to (6).

## Example 10

## Preparation of Electrophotographic Rollers 10-1 to 10-3

15 Electrophotographic rollers 10-1 to 10-3 were prepared in the same manner as in the electrophotographic roller 1-1 according to Example 1 except that the elastic rollers 2-1, 4-1 and 3-1 were used, and subjected to Evaluations (1) to (6).

## Example 11

## Preparation of Electrophotographic Roller 11

20 An electrophotographic roller 11 was prepared in the same manner as in the electrophotographic roller 2-1 according to Example 2 except that the elastic roller 3-2 was used, and subjected to Evaluations (1) to (6).

## Example 12

## Preparation of Electrophotographic Rollers 12-1 to 12-2

25 Electrophotographic rollers 12-1 to 12-2 were prepared in the same manner as in the electrophotographic roller 3-1 according to Example 3 except that the elastic rollers 4-2 and 2-2 were used, and subjected to Evaluations (1) to (6).

## Example 14

## Preparation of Electrophotographic Roller 14

30 An electrophotographic roller 14 was prepared in the same manner as in the electrophotographic roller 4-1 according to Example 4 except that the elastic roller 3-1 was used, and subjected to Evaluations (1) to (6).

## Example 16

## Preparation of Electrophotographic Rollers 16-1 to 16-2

35 Electrophotographic rollers 16-1 to 16-2 were prepared in the same manner as in the electrophotographic roller 4-1 according to Example 4 except that the elastic rollers 2-2 and 4-3 were used, and subjected to Evaluations (1) to (6).

## Example 17

## Preparation of Electrophotographic Roller 17

40 Electrophotographic rollers 17-1 to 17-2 were prepared in the same manner as in the electrophotographic roller 5-1

17

according to Example 5 except that the elastic roller 2-3 was used, and subjected to Evaluations (1) to (6).

## Example 18

## Preparation of Electrophotographic Rollers 18-1 to 18-2

Electrophotographic rollers 18-1 to 18-2 were prepared in the same manner as in the electrophotographic roller 3-1 according to Example 3 except that the elastic rollers 3-3 and 4-3 were used, and subjected to Evaluations (1) to (6).

## Example 9

## Preparation of Electrophotographic Roller 9-1

20 parts of by mass of isopropanol and 500 parts by mass of water were added based on 100 parts by mass of a mixture of titanium tetraisopropoxide and titanium tetra-octadecyloxide (=1/1, in molar ratio of Ti atoms), and heated and mixed at 150° C. for 2 hours. After cooling, the solution was charged into a dipping apparatus, the elastic roller 1-1 was dipped in the apparatus, pulled up, then air-dried for 60 minutes, and thereafter heated at a temperature of 180° C. for 5 hours, thereby producing a surface layer having a thickness of 100 nm. An electrophotographic roller 9-1 was thus prepared and subjected to Evaluations (1) to (6).

## Preparation of Electrophotographic Roller 9-2

An electrophotographic roller 9-2 was prepared in the same manner as in the electrophotographic roller 9-1 except that the elastic roller 1-5 was used, and subjected to Evaluations (1) to (6).

## Example 13

## Preparation of Electrophotographic Roller 13

An electrophotographic roller 13 was prepared in the same manner as in the electrophotographic roller 9-1 except that the mixture of titanium tetraisopropoxide and titanium tetra-octadecyloxide (=1/1) was changed to a mixture of titanium tetra-n-butoxide and titanium tetra-2-ethyl hexoxide (=1/1, in molar ratio of Ti atoms), and subjected to Evaluations (1) to (6).

## Example 15

## Preparation of Electrophotographic Roller 15

An electrophotographic roller 15 was prepared in the same manner as in the electrophotographic roller 9-1 except that the elastic roller 1-6 was used and the mixture of titanium tetraisopropoxide and titanium tetra-octadecyloxide (=1/1) was changed to titanium tetra-2-ethyl hexoxide, and subjected to Evaluations (1) to (6).

## Comparative Example 1

## Preparation of Electrophotographic Roller C-1

The elastic roller 1-1 was prepared as an electrophotographic roller C-1 according to Comparative Example 1, and subjected to Evaluations (5) to (6).

18

## Comparative Example 2

## Preparation of Electrophotographic Roller C-2

5 The elastic roller 2-1 was prepared as an electrophotographic roller C-2 according to Comparative Example 2, and subjected to Evaluations (5) to (6).

## Comparative Example 3

## Preparation of Electrophotographic Roller C-3

The elastic roller 3-1 was prepared as an electrophotographic roller C-3 according to Comparative Example 3, and subjected to Evaluations (5) to (6).

## Comparative Example 4

## Preparation of Electrophotographic Roller C-4

20 The elastic roller 4-1 was prepared as an electrophotographic roller C-4 according to Comparative Example 4, and subjected to Evaluations (5) to (6).

## Comparative Example 5

## Preparation of Electrophotographic Roller C-5

25 After titanium oxide powders (trade name: R-820, Ishihara Sangyo Kaisha, Ltd.) were sprinkled while rotating the elastic roller 1-1 in the circumferential direction, excessive titanium oxide powders were removed by an air gun to thereby prepare an electrophotographic roller C-5 in which the titanium oxide powders were supported on the surface of the elastic roller, and the electrophotographic roller C-5 was subjected to Evaluations (1) and (5) to (6).

## Comparative Example 6

## Preparation of Electrophotographic Roller C-6

30 A surface layer containing a titanium oxide film was formed on the surface of the elastic roller 1-1 by sputtering to thereby prepare an electrophotographic roller C-6, which was subjected to Evaluations (1), (5) and (6).

## Comparative Example 7

## Preparation of Electrophotographic Roller C-7

35 The elastic roller 1-1 was set in a CVD apparatus illustrated in FIG. 4, and the inside of a chamber was evacuated until reaching 2 Pa by a vacuum pump. Then, while tetramethyldisiloxane and oxygen were introduced into the chamber at a flow rate of 20 cm<sup>3</sup>/sec and at a flow rate of 100 cm<sup>3</sup>/sec, respectively, and the elastic roller 1-1 was rotated at a rotation number of 20 rpm, a 200 W of power at a frequency of 13.56 MHz was supplied between plate electrodes by a high-frequency power source to generate plasma between the electrodes. Such a state was maintained for 120 seconds to thereby form a surface layer containing a silica film on the periphery of the elastic roller 1-1. An electrophotographic roller C-7 was thus obtained. The electrophotographic roller C-7 was subjected to Evaluations (1) and (3) to (6).

40 With respect to Examples 1 to 18 described above, the evaluation results are shown in Table 11-1 and Table 11-2. In addition, the results of Comparative Examples 1 to 7 are shown in Table 12.

TABLE 11-1

|          |            | Evaluations |             |                |                                    |                   |       |         |         |                          |
|----------|------------|-------------|-------------|----------------|------------------------------------|-------------------|-------|---------|---------|--------------------------|
| Electro- | (1)        | photo-      | Presence of | Presence of    | (3)                                | (4)               | (5)-1 | (5)-2   | (6)-1   | (6)-2                    |
| graphic  | structural | Roller      | structural  | unit according | Surface                            | Vp/Ve             | Ghost | Filming | Fogging | Scraping                 |
|          |            | No.         |             |                | resistance<br>( $\Omega/\square$ ) |                   |       |         |         | resistance<br>of surface |
| Examples | 1          | 1-1         | Yes         | Yes            | 3                                  | $8.0 \times 10^7$ | 0.1   | A       | A       | A                        |
|          |            | 1-2         | Yes         | Yes            |                                    | 5                 | A     | A       | A       | A                        |
|          |            | 1-3         | Yes         | Yes            |                                    | 10                | A     | A       | A       | A                        |
|          | 2          | 2-1         | Yes         | Yes            | 4                                  | $2.2 \times 10^7$ | 0.1   | A       | A       | A                        |
|          |            | 2-2         | Yes         | Yes            |                                    | 5                 | A     | A       | A       | A                        |
|          |            | 2-3         | Yes         | Yes            |                                    | 10                | A     | A       | A       | A                        |
|          | 3          | 3-1         | Yes         | Yes            | 6                                  | $1.3 \times 10^8$ | 0.1   | A       | A       | A                        |
|          |            | 3-2         | Yes         | Yes            |                                    | 5                 | A     | A       | A       | A                        |
|          |            | 3-3         | Yes         | Yes            |                                    | 10                | A     | A       | A       | A                        |
|          | 4          | 4-1         | Yes         | Yes            | 8                                  | $4.5 \times 10^7$ | 0.1   | A       | A       | B                        |
|          |            | 4-2         | Yes         | Yes            |                                    | 5                 | A     | A       | A       | B                        |
|          |            | 4-3         | Yes         | Yes            |                                    | 10                | A     | A       | A       | B                        |
|          | 5          | 5-1         | Yes         | Yes            | 2                                  | $5.9 \times 10^7$ | 0.1   | A       | B       | A                        |
|          |            | 5-2         | Yes         | Yes            |                                    | 5                 | A     | B       | A       | A                        |
|          |            | 5-3         | Yes         | Yes            |                                    | 10                | A     | B       | A       | A                        |
|          | 6          | 6-1         | Yes         | Yes            | 3                                  | $8.0 \times 10^7$ | 0.1   | A       | A       | B                        |
|          |            | 6-2         | Yes         | Yes            |                                    | 11                | B     | A       | A       | A                        |
|          | 7          | 7-1         | Yes         | Yes            | 6                                  | $1.3 \times 10^8$ | 0.1   | A       | A       | B                        |
|          |            | 7-2         | Yes         | Yes            |                                    | 11                | B     | A       | A       | A                        |
|          | 8          | 8-1         | Yes         | Yes            | 8                                  | $4.5 \times 10^7$ | 0.05  | A       | A       | B                        |
|          |            | 8-2         | Yes         | Yes            |                                    | 11                | B     | A       | A       | A                        |
|          | 9          | 9-1         | Yes         | Yes            | 2                                  | $7.4 \times 10^8$ | 0.1   | A       | A       | C                        |
|          |            | 9-2         | Yes         | Yes            |                                    | 10                | A     | A       | A       | C                        |
|          | 10         | 10-1        | Yes         | Yes            | 3                                  | $8.0 \times 10^7$ | 0.1   | A       | A       | A                        |
|          |            | 10-2        | Yes         | Yes            |                                    | 5                 | A     | A       | A       | A                        |
|          |            | 10-3        | Yes         | Yes            |                                    | 10                | A     | A       | A       | A                        |

TABLE 11-2

|          |            | Evaluations |             |                |                                    |                   |       |         |         |                          |
|----------|------------|-------------|-------------|----------------|------------------------------------|-------------------|-------|---------|---------|--------------------------|
| Electro- | (1)        | photo-      | Presence of | Presence of    | (3)                                | (4)               | (5)-1 | (5)-2   | (6)-1   | (6)-2                    |
| graphic  | structural | Roller      | structural  | unit according | Surface                            | Vp/Ve             | Ghost | Filming | Fogging | Scraping                 |
|          |            | No.         |             |                | resistance<br>( $\Omega/\square$ ) |                   |       |         |         | resistance<br>of surface |
| Examples | 11         | 11          | Yes         | Yes            | 4                                  | $2.2 \times 10^7$ | 5     | A       | A       | A                        |
|          | 12         | 12-1        | Yes         | Yes            | 6                                  | $1.3 \times 10^8$ | 10    | A       | A       | A                        |
|          |            | 12-2        | Yes         | Yes            |                                    | 5                 | A     | A       | A       | A                        |
|          | 13         | 13          | Yes         | Yes            | 6                                  | $8.0 \times 10^9$ | 0.1   | A       | A       | A                        |
|          | 14         | 14          | Yes         | Yes            | 8                                  | $4.5 \times 10^7$ | 10    | A       | A       | B                        |
|          | 15         | 15          | Yes         | Yes            |                                    | $2.8 \times 10^9$ | 7     | A       | A       | B                        |
|          | 16         | 16-1        | Yes         | Yes            | 8                                  | $4.5 \times 10^7$ | 5     | A       | A       | B                        |
|          |            | 16-2        | Yes         | Yes            |                                    |                   | 0.1   | A       | A       | B                        |
|          | 17         | 17          | Yes         | Yes            | 2                                  | $5.9 \times 10^7$ | 5     | A       | B       | A                        |
|          | 18         | 18-1        | Yes         | Yes            | 6                                  | $1.3 \times 10^8$ | 11    | B       | A       | A                        |
|          |            | 18-2        | Yes         | Yes            |                                    |                   | 0.1   | A       | B       | A                        |

TABLE 12

|             |            | Evaluations |             |                |                                    |       |       |         |         |                          |
|-------------|------------|-------------|-------------|----------------|------------------------------------|-------|-------|---------|---------|--------------------------|
| Electro-    | (1)        | photo-      | Presence of | Presence of    | (3)                                | (4)   | (5)-1 | (5)-2   | (6)-1   | (6)-2                    |
| graphic     | structural | Roller      | structural  | unit according | Surface                            | Vp/Ve | Ghost | Filming | Fogging | Scraping                 |
|             |            | No.         |             |                | resistance<br>( $\Omega/\square$ ) |       |       |         |         | resistance<br>of surface |
| Comparative | 1          | C-1         | No          | No             | —                                  | —     | —     | A       | A       | B                        |
| Examples    | 2          | C-2         | No          | No             | —                                  | —     | —     | A       | A       | D                        |
|             |            |             |             |                |                                    |       |       | C       |         |                          |
|             |            |             |             |                |                                    |       |       | D       |         |                          |

TABLE 12-continued

| Electro-<br>photo-<br>graphic<br>Roller<br>No. | Evaluations                                                            |                                                                        |     |                      |     |       |       |       |       |
|------------------------------------------------|------------------------------------------------------------------------|------------------------------------------------------------------------|-----|----------------------|-----|-------|-------|-------|-------|
|                                                | (1)                                                                    |                                                                        | (2) | (3)                  | (4) | (5)-1 | (5)-2 | (6)-1 | (6)-2 |
|                                                | Presence<br>of<br>structural<br>unit<br>according<br>to formula<br>(1) | Presence<br>of<br>structural<br>unit<br>according<br>to formula<br>(2) |     |                      |     |       |       |       |       |
| 3 C-3                                          | No                                                                     | No                                                                     | —   | —                    | —   | A     | A     | C     | D     |
| 4 C-4                                          | No                                                                     | No                                                                     | —   | —                    | —   | A     | A     | C     | D     |
| 5 C-5                                          | Yes                                                                    | No                                                                     | —   | —                    | —   | A     | B     | B     | D     |
| 6 C-6                                          | Yes                                                                    | No                                                                     | —   | —                    | —   | B     | C     | B     | A     |
| 7 C-7                                          | No                                                                     | No                                                                     | —   | $3.0 \times 10^{15}$ | 30  | C     | A     | A     | A     |

The electrophotographic rollers prepared in Examples 1 to 18 have the titanium oxide film in which the surface layer contains both chemical bonds represented by the formula (1) and the formula (2).

The titanium oxide film containing the bond represented by the formula (2) has a smaller number of bonds between atoms than the titanium oxide film containing only the chemical bond represented by the formula (1), and thus is a flexible film. Therefore, even in the case where the electrophotographic roller according to each Example was used as the developing roller, a toner was fixed to the surface with difficulty, and generation of the filming was suppressed.

In addition, even in the case where the electrophotographic roller according to each Example was used as the developing roller, no scraping of the surface layer was observed, and ghost performance and fogging performance were favorable because the surface layer was conductive.

On the other hand, the electrophotographic rollers C-1 to C-4 according to Comparative Examples 1 to 4 were relatively inferior in durability because the surfaces were made of the resin or rubber derived from the elastic layer, and in the case where the electrophotographic rollers were used as the developing roller, scraping was observed on the surfaces due to rubbing friction with a photosensitive drum and a developer regulating member.

When the electrophotographic roller C-5 according to Comparative Example 5, in which the titanium oxide powders were adhered on the surface, was used as the developing roller, the titanium oxide powders were peeled off from the surface of the elastic layer and the surface of the elastic layer was exposed, resulting in scraping observed on the surface. Furthermore, since no smoothness was on the surface, a toner likely remained on the surface of the developing roller to thereby likely allow the toner to be fixed, and filming was observed.

Since the electrophotographic roller according to Comparative Example 6, having a surface layer containing a titanium oxide film having no chemical bond represented by the formula (2) as the surface layer, had a hard surface layer, filming of a toner was generated.

Since the electrophotographic roller C-7 according to Comparative Example 7, having a surface layer containing a silica film, had an insulating surface layer, the surface potential was high and a ghost image was observed in the electrophotographic image.

As described above, even when the electrophotographic roller according to the present invention is used as the developing roller for a long period of time, the surface layer is hardly scraped. In addition, since the titanium oxide film according to the present invention has conductivity, a ghost image is hardly generated. In addition, since the titanium

oxide film according to the present invention is more flexible than the titanium oxide film containing only the chemical bond represented by the formula (1), the titanium oxide film according to the present invention causes deterioration of a toner with difficulty and is conducive to stably forming a high quality electrophotographic image for a long period.

#### Example 19

The same electrophotographic roller as the electrophotographic roller 10-1 according to Example 10 was prepared, and defined as an electrophotographic roller 19 according to the present Example. The electrophotographic roller 19 had the same results of Evaluations (1) to (4) as the results for the electrophotographic roller 10-1, and thus was not subjected to Evaluations (1) to (4) but was subjected to the following Evaluation (7).

##### <Evaluation (7)>

The electrophotographic roller 19 was mounted as a charging roller to a process cartridge for a color laser printer (trade name: LBP7700C (altered machine), manufactured by Canon Inc.). The process cartridge was loaded to the color laser printer. The laser printer was used to output 20,000 sheets of electrophotographic images under an environment of a temperature of 15°C and a relative humidity of 10%. The electrophotographic images were images in which 4-point size letters of alphabet "E" were printed on an A4-size sheet so that the printing percentage was 1%. Subsequently, two halftone images, one having a density different from a density of the other, were each output one by one. Herein, one halftone used had a density of 0.4 and the other had a density of 0.7 as measured by a spectral densitometer: X-Rite 504 (trade name, S.D.G.K.K.).

The process cartridge was taken out from the electrophotographic apparatus after forming the halftone image, the electrophotographic roller 19 was taken out from the process cartridge, and the surface was observed by an optical microscope at a magnification of 500 times in 20 points. Then, the presence of an adhered substance observed and the size of the adhered substance were evaluated according to the criteria described in the following Table 13.

TABLE 13

| Rank | Criteria                                                                                                                                                                                     |
|------|----------------------------------------------------------------------------------------------------------------------------------------------------------------------------------------------|
| A    | No adhered substance having a size of 10 $\mu\text{m}$ or more was observed.                                                                                                                 |
| B    | No adhered substance having a size of 50 $\mu\text{m}$ or more was observed, but an adhered substance having a size of 10 $\mu\text{m}$ or more and less than 50 $\mu\text{m}$ was observed. |

## 23

TABLE 13-continued

| Rank | Criteria                                                                     |
|------|------------------------------------------------------------------------------|
| C    | An adhered substance having a size of 50 $\mu\text{m}$ or more was observed. |

The presence of a stripe due to uneven charging of the charging roller was visually observed for the two sheets of halftone images obtained as described above, and evaluated according to the criteria described in the following Table 14.

TABLE 14

| Rank | Criteria                                                  |
|------|-----------------------------------------------------------|
| A    | No stripe was observed for both the two halftone images.  |
| B    | A stripe was observed for one of the two halftone images. |
| C    | A stripe was observed for both the two halftone images.   |

## Example 20

An electrophotographic roller 20 was prepared in the same manner as in the electrophotographic roller 9-1 according to Example 9 except that the elastic roller 3-1 was used and

5 An electrophotographic roller 23 was prepared in the same manner as in the electrophotographic roller 19 according to Example 19 except that the elastic roller 6 was used, and subjected to Evaluations (1) to (4) and (7).

## Example 24

An electrophotographic roller 24 was prepared in the same 10 manner as in the electrophotographic roller 20 according to Example 20 except that the elastic roller 7 was used, and subjected to Evaluations (1) to (4) and (7).

## Comparative Example 8

15 A surface layer containing a titanium oxide film was formed on the periphery of the elastic roller 2-1 by sputtering to thereby prepare an electrophotographic roller C-8, which was subjected to Evaluations (1) and (7).

## Comparative Example 9

An electrophotographic roller C-9 was prepared in the same manner as in the electrophotographic roller C-7 according to Comparative Example 7 except that the elastic roller 7 was used, and subjected to Evaluations (1), (3), (4) and (7).

The evaluation results of Examples 19 to 24 and Comparative Examples 8 to 9 described above are shown in Table 15.

TABLE 15

|                      | Evaluations                     |                        |                      |      |      |                      |                                        |       |                               |
|----------------------|---------------------------------|------------------------|----------------------|------|------|----------------------|----------------------------------------|-------|-------------------------------|
|                      |                                 |                        |                      |      |      |                      |                                        |       |                               |
|                      | (1)                             |                        |                      |      |      |                      | (7)                                    |       |                               |
| Examples             | Presence of Electro- structural | Presence of structural | photo- graphic       | unit | unit | (3)                  | Surface resistance                     | (4)   | Stripe due to uneven charging |
|                      | Roller No.                      | according to formula   | according to formula | (1)  | (2)  | (2)                  | Cc-<br>c/Oc-o<br>( $\Omega/\text{m}$ ) | Vp/Ve | Adhered substance             |
| Examples             | 19                              | 19                     | Yes                  | Yes  | 3    | $8.0 \times 10^7$    | 0.1                                    | A     | A                             |
|                      | 20                              | 20                     | Yes                  | Yes  | 4    | $8.4 \times 10^9$    | 5                                      | B     | A                             |
|                      | 21                              | 21                     | Yes                  | Yes  | 3    | $2.2 \times 10^7$    | 10                                     | A     | A                             |
|                      | 22                              | 22                     | Yes                  | Yes  | 4    | $6.2 \times 10^9$    | 0.1                                    | A     | A                             |
|                      | 23                              | 23                     | Yes                  | Yes  | 3    | $8.0 \times 10^7$    | 5                                      | A     | A                             |
|                      | 24                              | 24                     | Yes                  | Yes  | 4    | $5.9 \times 10^7$    | 10                                     | B     | A                             |
| Comparative Examples | 8                               | C-8                    | Yes                  | No   | —    | —                    | —                                      | C     | B                             |
|                      | 9                               | C-9                    | No                   | No   | —    | $3.0 \times 10^{15}$ | 30                                     | B     | C                             |

titanium tetraethoxide was used as a raw material gas, and subjected to Evaluations (1) to (4) and Evaluation (7).

## Example 21

An electrophotographic roller 21 was prepared in the same manner as in the electrophotographic roller 1-1 according to Example 1 except that the elastic roller 4-1 was used and titanium tetra-n-propoxide was used as a raw material gas, and subjected to Evaluations (1) to (4) and (7).

## Example 22

An electrophotographic roller 22 was prepared in the same manner as in the electrophotographic roller 9-1 according to Example 9 except that the elastic roller 5 was used and titanium tetra-n-propoxide was used as a raw material gas, and subjected to Evaluations (1) to (4) and (7).

50 In the case where the electrophotographic roller according to the present invention is used as the charging roller, the surface layer contains the alkoxy-modified titanium oxide film to thereby suppress adhesion of foreign substances on the surface of the charging roller. Therefore, generation of uneven charging on the electrophotographic photoreceptor due to the charging roller could be suppressed, and as a result, generation of the stripe on the electrophotographic image due to the uneven charging could be suppressed.

55 On the other hand, the electrophotographic roller C-8 according to Comparative Example 8, having a surface layer containing a titanium oxide film having no chemical bond represented by the formula (2) as the surface layer, had a high elastic modulus to thereby have a higher contact pressure with the photosensitive drum and thus was likely adhered to an external additive for a toner, and an adhered substance having a size of 50  $\mu\text{m}$  or more was observed on the surface of the 60 charging roller.

65 The electrophotographic roller C-9 according to Comparative Example 9, having a surface layer containing a silica film,

25

had a high surface potential, and thus an external additive for a toner was electrostatically adhered on the surface. In addition, uneven adhesion and a high surface potential were combined with each other to generate uneven surface potential in the circumferential direction of the charging roller and to generate uneven charging in the electrophotographic photoreceptor, resulting in generating the stripe due to the uneven charging in the electrophotographic image.

From the foregoing, it has been found that in the case where the electrophotographic roller according to the present invention is used as the charging roller, adhesion of foreign substances on the surface of the charging roller and the stripe due to the uneven charging can be suppressed.

While the present invention has been described with reference to exemplary embodiments, it is to be understood that the invention is not limited to the disclosed exemplary embodiments. The scope of the following claims is to be accorded the broadest interpretation so as to encompass all such modifications and equivalent structures and functions.

This application claims the benefit of Japanese Patent Application No. 2011-133744, filed Jun. 15, 2011, which is hereby incorporated by reference herein in its entirety.

What is claimed is:

1. An electrophotographic member comprising:  
a mandrel,  
an elastic layer, and  
a surface layer;

26

wherein,

the surface layer comprises a titanium oxide film having chemical bonds represented by the following formula (1) and formula (2)



Formula (1)



Formula (2)

wherein an abundance ratio ( $C_{C-C}/O_{C-O}$ ) is 3 or more and 8 or less, wherein  $O_{C-O}$  represents an abundance ratio of an oxygen atom bound to a carbon atom, ( $O_{C-O}$ ), and  $C_{C-C}$  represents an abundance ratio of a carbon atom bound to a carbon atom, ( $C_{C-C}$ ), in the titanium oxide film.

2. The electrophotographic member according to claim 1, 15 wherein the titanium oxide film comprises a hydrolytic condensate of titanium tetraalkoxide represented by the following formula (3):



Formula (3)

(in the formula (3), R represents a linear or branched-chain alkyl group having 2 to 18 carbon atoms).

3. A process cartridge provided with an electrophotographic member according to claim 1, and configured to be attachable to and removable from a main body of an electrophotographic apparatus.

4. An electrophotographic apparatus provided with an electrophotographic member according to claim 1.

\* \* \* \* \*